

## UNITED STATES PATENT OFFICE

2,635,709

## ADSORPTION OF OLEFINS BY PETROLEUM COKE

Francis M. Archibald and William A. Konrad,  
Elizabeth, and Roy E. D. Haney, Westfield,  
N. J., assignors to Standard Oil Development  
Company, a corporation of Delaware

No Drawing. Application August 22, 1949,  
Serial No. 111,772

6 Claims. (Cl. 183—114.2)

1

This invention relates to the selective adsorption of gaseous olefin hydrocarbons from mixtures thereof with gaseous paraffin hydrocarbons by means of selective adsorption of the olefin when the hydrocarbon mixture containing olefins and paraffins, including normal and iso-paraffins, is brought into contact with a petroleum coke the nature of which is hereinafter explained.

It is well known that activated carbons possess the property of separating gaseous hydrocarbons according to molecular weight, the selectivity in separating a binary mixture being for the higher molecular weight component. It has now been discovered that coke recovered from the calcining of petroleum acid sludges displays on the contrary a selective affinity for olefin, or unsaturated hydrocarbons in preference to the paraffin or saturated hydrocarbons. It has also been found that this selectivity and also the capacity of the coke for the olefin can be enhanced by treating such a coke with nitrogen at a temperature of 1600—1800° F. for a period of 15 minutes to 2 hours, preferably 20 to 60 minutes.

Acid sludges are produced as a result of various petroleum refining operations particularly the sulfuric acid treatment of gasoline, lubricating oils and higher-boiling petroleum distillates particularly phenol extracted oil from which the so-called white oils are prepared by treatment with fuming sulfuric acid or  $\text{SO}_3$ . The resulting acid layers from the above treating operations vary in character depending upon the severity of the acid treatment but in general consist of a carbonaceous residue admixed with unreacted sulfuric acid, sulfonic acids, sulfur derivatives and water from which a tarry residue called a sludge is obtained upon the settling of the acid layer.

The activated petroleum coke which is employed in this invention is prepared as follows: The tarry sludge is introduced into a decomposition zone. In the decomposition zone the sludge is carbonized by contacting it in the absence of air with a mass of hot coke maintained with continuous stirring at a temperature of 400° F. to about 750° F., preferably about 600° F. to 700° F. for a period of time sufficient to distill therefrom the bulk of the volatile matter present in the sludge. During the carbonization the weight of coke to sludge is maintained at a ratio from about 2:1 to about 6:1. The carbonized sludge is then transferred to a kiln where it is partially burned with air at a temperature of 650° F. to 1200° F., preferably 1000° F. to 1200° F. for a period of time depending upon the type of coke desired, generally 5 to 25 minutes. The bulk of the resulting hot coke is recycled to the decomposition zone to maintain the mass of coke therein and to supply the necessary heat for the

5 carbonization, the balance of the coke is removed as the desired product which is cooled and comminuted to desired size. About seven lbs. of hot coke are recycled to the decomposition zone for each 1 lb. of coke removed as product which is known as petroleum coke. It is this product which has been found, contrary to the prior art teaching on carbon adsorbents, to have selective affinity for olefin hydrocarbons in preference to paraffin hydrocarbons.

10 The invention is illustrated by the following data obtained from experiments in which gaseous mixtures of ethylene and propane and of ethylene and ethane were passed over a mass of petroleum coke until equilibrium was established. The coke was desorbed by heating under vacuum or by treating at elevated temperature with an inert gas such as nitrogen, helium, etc. Steam is not to be employed if it is desired to reemploy the coke in the adsorption process because it has been found that the action of steam destroys the selective affinity of the coke for olefins and reverts it to its normal selectivity for paraffins or higher molecular weight hydrocarbon. However, steam may be employed as the desorbing medium if it is desired to re-use the desorbed coke for other purposes such as the normal gaseous adsorption operation wherein paraffins or higher molecular weight hydrocarbons are selectively adsorbed in preference to olefins or lower molecular weight hydrocarbons. The steam-stripped carbon can also be employed for other uses not involving hydrocarbon separation, e. g., purification of water, sugar and medicinals by removal of color and odor therefrom.

TABLE I  
Adsorption of gaseous hydrocarbons on  
petroleum coke

|                                                                          | Ethylene<br>from Pro-<br>pane | Ethylene<br>from Eth-<br>ane |
|--------------------------------------------------------------------------|-------------------------------|------------------------------|
| 45 Adsorptive Capacity (millimols/gm.)                                   | 1.06                          | 1.77                         |
| Percent $\text{C}_2\text{H}_4$ in Feed Gas                               | 45.92                         | 51.52                        |
| Percent $\text{C}_2\text{H}_4$ in Residual Gas                           | 33.55                         | 49.09                        |
| Percent $\text{C}_2\text{H}_4$ in Adsorbate in equilibrium<br>with vapor | 79.71                         | 55.03                        |
| Separation Factor, $\alpha^1$                                            | 2.7.78                        | 1.27                         |

50  $^1 \alpha = \frac{(\text{Conc. of less adsorbed comp. in vapor})}{(\text{Conc. of more adsorbed comp. in vapor})} \times$

$(\text{Conc. of more adsorbed comp. in adsorbate})$   
 $(\text{Conc. of less adsorbed comp. in adsorbate})$

55 55  $^2$  Indicates the petroleum coke to be selective for the olefin component.

60 It has further been found that the action of petroleum coke in adsorbing olefin hydrocarbons is enhanced by treating the coke with nitrogen at a temperature of 1600° F. to 1800° F. for

a period of 15 minutes to 2 hours, preferably 20 minutes to 60 minutes.

Data obtained from similar runs employing the nitrogen-activated petroleum coke are as follows:

TABLE II

*Separation of ethylene-propane mixtures with petroleum coke heated to 1600° F. (approx. 15° F./min.) in a nitrogen atmosphere*

|                                                       |      |
|-------------------------------------------------------|------|
| Adsorption (millimols/gm.)                            | 1.2  |
| Percent C <sub>2</sub> H <sub>4</sub> in feed gas     | 42.9 |
| Percent C <sub>2</sub> H <sub>4</sub> in residual gas | 33.9 |
| Percent C <sub>2</sub> H <sub>4</sub> in adsorbate    | 79.0 |
| Separation factor, <i>a</i>                           | 7.34 |

It appears that the rate of adsorption is enhanced by the nitrogen treatment, i. e. to attain a given level of adsorption less time is required with the nitrogen-treated material since approximately 8-10% volatile material is liberated from the coke during this treating operation.

The desorption of the fat adsorbent with nitrogen may also serve at least in part as the activation step whereby the selectivity and capacity of the coke for olefins are enhanced.

The process is applicable to the adsorption-separation of the normally gaseous olefins, i. e. the C<sub>2</sub>-C<sub>5</sub> olefins, including ethylene, propylene, butenes, and amylanes. In general the adsorption is carried out at a temperature of 60-200° F., preferably 75-100° F. and at a pressure of 1-12 atmospheres, preferably 5-7 atmospheres. The desorption is carried out at temperatures in the range of 300-700° F., preferably 450-550° F., and at the same pressure as the adsorption step or lower.

By the term petroleum coke as employed in the appended claims is meant a coke prepared from petroleum acid sludges by the method previously described in this specification.

Having described the invention, what is claimed as new and what is desired to be secured by Letters Patent is:

1. A process for the separation of ethylene from a mixture comprising ethylene and propane which comprises contacting the mixture with a coke prepared by calcining a sulfuric acid-petroleum whereby the ethylene is selectively adsorbed and thereafter recovering ethylene from the petroleum coke.

2. A process for the separation of ethylene from a mixture comprising ethylene and propane which comprises contacting the mixture with a petroleum coke prepared by calcining a sulfuric acid-petroleum which coke has been further activated by treatment with nitrogen at 1600° F. to 1800° F. whereby the ethylene is selectively adsorbed and thereafter recovering ethylene from the petroleum coke.

3. An activated carbon adaptable for the preferential adsorption of an olefin from a gaseous

hydrocarbon mixture of an olefin hydrocarbon and a paraffin hydrocarbon in which the paraffin contains a greater number of carbon atoms than the olefin, prepared by calcining a sulfuric acid-petroleum sludge to form a coke and thereafter treating the coke with nitrogen at a temperature of 1600° F. to 1800° F.

4. A process for the separation of an olefin from a gaseous hydrocarbon mixture of an olefin hydrocarbon and a paraffin hydrocarbon in which the paraffin contains a greater number of carbon atoms than the olefin which comprises contacting the mixture with a coke prepared by calcining a sulfuric acid-petroleum sludge whereby the olefin is selectively adsorbed, and thereafter recovering the adsorbed olefin from the coke.

5. A process for the separation of an olefin from a gaseous hydrocarbon mixture of an olefin hydrocarbon and a paraffin hydrocarbon in which the paraffin contains a greater number of carbon atoms than the olefin, which comprises contacting the mixture with a coke prepared by calcining a sulfuric acid-petroleum sludge and subsequently contacting the coke with nitrogen at 1600° F. to 1800° F., whereby the olefin hydrocarbon is selectively adsorbed, and thereafter recovering the adsorbed olefin from the coke.

6. A process for the preparation of an activated carbon adaptable for the preferential adsorption of an olefin from a gaseous hydrocarbon mixture of an olefin hydrocarbon and a paraffin hydrocarbon in which the paraffin contains a greater number of carbon atoms than the olefin which comprises contacting petroleum-sulfuric acid sludge coke with nitrogen at a temperature of 1600° F. to 1800° F.

FRANCIS M. ARCHIBALD.  
WILLIAM A. KONRAD.  
ROY E. D. HANEY.

## References Cited in the file of this patent

## UNITED STATES PATENTS

|    | Number    | Name            | Date           |
|----|-----------|-----------------|----------------|
| 45 | 1,452,322 | Stewart         | Apr. 17, 1923  |
|    | 1,865,422 | Askenasy        | July 5, 1932   |
|    | 1,872,080 | Harris          | Aug. 16, 1932  |
|    | 2,296,438 | Hassler et al.  | Sept. 22, 1942 |
| 50 | 2,384,311 | Kearby          | Sept. 4, 1945  |
|    | 2,393,214 | Andrews         | Jan. 15, 1946  |
|    | 2,470,339 | Claussen et al. | May 17, 1949   |
|    | 2,476,472 | Arnold et al.   | July 19, 1949  |
|    | 2,485,352 | Bircher         | Oct. 18, 1949  |
| 55 | 2,493,911 | Brandt          | Jan. 10, 1950  |
|    | 2,519,344 | Berg            | Aug. 22, 1950  |
|    | 2,519,874 | Berg            | Aug. 22, 1950  |

## FOREIGN PATENTS

|    | Number  | Country       | Date          |
|----|---------|---------------|---------------|
| 60 | 586,766 | Great Britain | Mar. 31, 1947 |
|    | 597,895 | Great Britain | Feb. 5, 1948  |